

# UNITED STATES PATENT OFFICE.

EDWARD D. GLEASON, OF NEW YORK, N. Y., ASSIGNOR, BY MESNE ASSIGNMENTS, TO NEU-METALS AND PROCESS COMPANY, OF LONG ISLAND CITY, NEW YORK, A CORPORATION OF NEW YORK.

## ALLOY.

1,093,557.

Specification of Letters Patent.

Patented Apr. 14, 1914.

No Drawing.

Application filed February 18, 1913. Serial No. 749,109.

To all whom it may concern:

Be it known that I, EDWARD D. GLEASON, a citizen of the United States, residing in Brooklyn, in the county of Kings, city and State of New York, have invented a certain new and useful Improvement in Alloys, whereof the following is a specification.

It is the ultimate object of my invention to provide boiler and condenser tubes of homogeneous metal capable of resisting corrosion, but my improved alloy is not only capable of resisting the corrosive action of water and steam but is also capable of resisting the action of sulfuric and nitric acids and other corrosive liquids, and consequently may be employed for other structures than such tubes. Said alloy is about the color of platinum and has a coefficient of expansion, by heat, approximately that of glass. I find that the useful properties aforesaid are characteristic of alloys within the following range of proportions by weight:—

|    |          |                 |
|----|----------|-----------------|
| 25 | Iron     | 80 to 120 parts |
|    | Nickel   | 80 to 120 parts |
|    | Copper   | 1 part          |
|    | Aluminum | 4 parts.        |

I find it preferable to employ Swedish iron in making such alloys and a typical example, having the useful properties above stated, is as follows:—

|    |              |           |
|----|--------------|-----------|
| 35 | Swedish iron | 110 parts |
|    | Nickel       | 90 parts  |
|    | Copper       | 1 part    |
|    | Aluminum     | 4 parts.  |

It is to be noted that ordinary alloys including iron-nickel-copper are objectionable 40 in that casting and cooling the same usually

results in separation of said metals and formation of hard nodules throughout the mass of the alloy. Consequently, it has been the practice hitherto to include in such alloys manganese, magnesium, or some other de- 45 oxidizing agent, and more or less carbon; the strength of such ordinary alloys being apparently dependent upon the amount of carbon retained therein. However, alloys within the proportions above stated may be 50 made without the inclusion of the de-oxidizing agents aforesaid, and without regard to carbon and are not only homogeneous but are so ductile that they may be readily rolled to sheet or drawn to tube and wire 55 forms.

Alloys in accordance with my invention do not require any special method or means of manufacture, and ordinary methods and means may be employed.

I do not desire to limit myself to the precise proportions herein set forth as it is obvious that various modifications may be made therein without departing from the essential features of my invention as defined in the appended claims.

I claim:—

1. An alloy comprising iron 80 to 120 parts, nickel 80 to 120 parts, copper 1 part and aluminum 4 parts.

2. An alloy comprising Swedish iron 110 parts, nickel 90 parts, copper 1 part, and aluminum 4 parts.

In testimony whereof, I have hereunto signed my name at Philadelphia, Pa., this 75 17th day of February, 1913.

EDWARD D. GLEASON.

Witnesses:

ARTHUR E. PAIGE,  
ANNA ISRAELVITZ.